

## UNITED STATES PATENT OFFICE

1,925,564

PROCESS FOR THE RECLAMATION OF  
FILM SCRAP WITH PERMANGANATE  
SOLUTIONSThomas F. Murray, Jr., and Cyril J. Staud,  
Rochester, N. Y., assignors to Eastman Kodak  
Company, Rochester, N. Y., a corporation of  
New YorkNo Drawing. Application May 24, 1930.  
Serial No. 455,450

4 Claims. (Cl. 8—2)

This invention relates to a process for the reclamation of photographic film scrap and more particularly to a process for reclaiming film scrap having a base of a cellulose derivative which 5 has been dyed.

In substantially all methods for the recovery of film scrap, the silver halide emulsion is first removed from the film scrap by soaking the scrap in hot water for a short length of time to loosen 10 the emulsion from the scrap. This leaves the film base or support, which may be composed of either cellulose nitrate or cellulose acetate. This film scrap base is then normally either (1) leached with an alcohol solution or (2) 15 bleached and then leached. The bleaching step has heretofore been accomplished with various compounds which liberate free chlorine, namely, calcium hypochlorite, sodium hypochlorite, hypochlorous acid, or combinations or equivalents thereof. In some instances this treatment is not entirely satisfactory for the reason 20 that the free chlorine, as well as the chloride, must be removed from the scrap before it can be utilized.

25 We have found that a good many of these seeming complications may be avoided if the film scrap from which the silver halide emulsion has been removed is bleached with a permanganate such as potassium or sodium permanganate, permanganic acid or a mixture of all or any of these.

The greatest disadvantage in connection with permanganate bleaching is, however, that the permanganates are more costly than the hypochlorites for the same weight of available 35 oxygen.

In certain industrial processes there are, however, large quantities of dilute acid permanganate liquors which cannot be longer used nor economically recovered but which, so far as their 40 oxidizing values are concerned, are just as useful as fresh solutions. These waste permanganate liquors occur, for instance, in the process whereby exposed Cine film is developed and re-developed by what is known as the reversal process. This liquor has a permanganate content of from about .1% to approximately 1%. When 45 used directly on film scrap base, however, these liquors are ineffective to completely remove the color therefrom even after several hours of treatment; some additional treatment was, therefore, found necessary.

We have discovered that these waste permanganate liquors may be utilized for the bleaching 50 of film scrap base and other scrap if the scrap

base is first leached with dilute alcohol, followed by bleaching with the dilute permanganate solutions mentioned above. For instance, dyed cellulose acetate film scrap from which the silver halide emulsion has been removed may be treated 60 in a 50% methyl alcohol solution for about three hours and then washed with water, after which the scrap is subjected to treatment with a waste permanganate solution of the character above described. It was found that after as short a 65 treatment as 15 minutes that the scrap was colorless.

Longer treatments up to one hour or even two hours or more may be desirable where a particularly deep color has to be removed. The temperature employed may be approximately room temperature, namely, from about 20 to 26 degrees centigrade. After the permanganate treatment, the scrap is removed and washed with water and then "cleared" in, for instance, an acidified sodium bisulfite solution prepared by dissolving 5 70 grams of sodium bisulphite in one liter of water and adding 5 cc of 35% hydrochloric acid or an equivalent quantity of sulfuric acid.

It will be understood that in the case of cellulose acetate film scrap base that the leaching solution may consist of either a methyl or ethyl alcohol mixture, and that the alcohol may be in the proportion of from 70 to 30 per cent alcohol to from 30 to 70 per cent of water. The sodium bisulfite solution is used merely to clarify the film scrap of any permanganate compound and may be a rather dilute solution mildly acidified. The product resulting from the permanganate oxidation may be removed by equivalents of sodium bisulphite such as oxalic acid, sodium nitrite, hydroxylamine, sodium hydrosulphite, sodium metabisulphite or other polythioic acids or their salts.

In the event that it is desired to reclaim film 95 scrap having a cellulose nitrate base the only precaution necessary is to not employ methyl alcohol in the leaching solution, it being desired, of course, not to employ in the leaching of either the cellulose nitrate or cellulose acetate base any 100 leaching solution which is a solvent for the film base.

When alcohol is employed for leaching cellulose acetate before bleaching, it performs a diversity of functions, among which may be mentioned: (1) removal of a portion of the dye present, if the same be alcohol soluble; (2) removal of any other alcohol soluble component of the material; (3) increasing the permeability of the 105 surface layers of the material resulting in more 110

ready penetrability of the cellulose acetate for bleaching solutions.

Also there are instances where it may be advantageous to employ alcohol for leaching cellulose acetate after bleaching. By so doing we have the advantage of (1) removal of the products of reaction; (2) removal of alcohol soluble components of the material; (3) removal of residual dye which was not acted upon during bleaching if such dyes be alcohol soluble. This leaching after bleaching need not be more fully set forth here as approximately the same procedure is followed as when leaching before bleaching except that the time of treatment need not be quite as long.

What has been stated above concerning alcohol is to be construed as equally applicable to other non-solvents which are suitable for this purpose and apparent to those skilled in the art.

It will thus be apparent that our invention is in fact two fold, namely, (1) the bleaching of dyed cellulosic derivative scrap and (2) the leaching of dyed cellulosic derivative scrap prior to the bleaching thereof, the bleaching being optionally followed by further leaching if desired. One is, of course, more or less of a specific subcombination of bleaching included in the broad concept of leaching and bleaching, as the two are quite apparently useful in connection with each other. Those claims appended hereto and directed to bleaching are not, of course, limited to a bleaching preceded by leaching as it may well be employed without previous leaching altho the latter is to be preferred. Also those claims directed more or less broadly to leaching and bleaching are not limited (unless so stated) to a bleaching step including the use of a permanganate as it will be quite apparent that previous leaching will make more easy the majority of bleaching processes such as those disclosed in applications of Charles E. Allen filed of even date, or even the usual hypochlorite or chlorine bleach as disclosed in the Middleton Patent #1,743,155.

Numerous other variations and modifications of the invention will occur to those skilled in the art, and it is intended that all modifications indicated above and which would occur to those skilled in the art shall be included within the spirit of this invention and the scope of the claims appended hereto. For instance, the process is equally applicable to any dyed cellulose derivative waste, such as dyed artificial silk waste which has a base of cellulose nitrate or acetate.

What we claim as our invention and desire to

be secured by Letters Patent of the United States is:

1. The process of reclaiming dyed cellulose derivative film scrap which comprises removing the alcohol soluble components of the scrap by leaching it with a 30-70% aqueous ethyl alcohol solution whereby such components are removed and the scrap is rendered porous, swollen and readily susceptible to further processing, washing the leached scrap to remove residual alcohol, decolorizing the washed material by subjecting it to the oxidizing action of an acid solution of permanganate containing 1-1% of permanganate and thereafter removing the oxidized material from the scrap. 80

2. The process of reclaiming dyed photographic cellulose acetate film scrap which comprises pre-treating the scrap to remove alcohol soluble components and to increase the permeability of the surface layers thereof by leaching with a 30-70% aqueous ethyl alcohol solution, washing the leached scrap with water to remove residual alcohol, decolorizing the washed scrap by subjecting it to the oxidizing action of a 1-1% solution of potassium permanganate, washing the bleached scrap with water and thereafter clearing the scrap from traces of unused permanganate by subjecting it to the reducing action of an acidified solution of sodium bisulphite. 95

3. The process of reclaiming dyed cellulose derivative scrap which comprises removing the alcohol soluble components of the scrap by leaching it with an alcohol which is non-solvent of the film scrap, whereby the alcohol soluble components of the scrap are removed and the scrap is rendered porous, swollen and readily susceptible to further processing, decolorizing the scrap by subjecting it to the oxidizing action of a bleaching solution and thereafter removing from the scrap the products of the oxidation. 105

4. The process of reclaiming dyed cellulose derivative scrap which comprises removing the alcohol soluble components of the scrap by leaching it with an aqueous alcohol which is non-solvent of the film scrap, whereby the alcohol soluble components of the scrap are removed and the scrap is rendered porous, swollen and readily susceptible to further processing, decolorizing the scrap by subjecting it to the oxidizing action of a permanganate solution and thereafter removing from the scrap the products of the oxidation. 120

THOMAS F. MURRAY, JR.  
CYRIL J. STAUD.

Patent No. 1,925,564.

September 5, 1933.

THOMAS F. MURRAY, JR., ET AL.

It is hereby certified that error appears in the printed specification of the above numbered patent requiring correction as follows: Page 2, line 79, claim 1, strike out the word "film"; and that the said Letters Patent should be read with this correction therein that the same may conform to the record of the case in the Patent Office.

Signed and sealed this 28th day of November, A. D. 1933.

F. M. Hopkins

(Seal)

Acting Commissioner of Patents.

ready penetrability of the cellulose acetate for bleaching solutions.

Also there are instances where it may be advantageous to employ alcohol for leaching cellulose acetate after bleaching. By so doing we have the advantage of (1) removal of the products of reaction; (2) removal of alcohol soluble components of the material; (3) removal of residual dye which was not acted upon during bleaching if such dyes be alcohol soluble. This leaching after bleaching need not be more fully set forth here as approximately the same procedure is followed as when leaching before bleaching except that the time of treatment need not be quite as long.

What has been stated above concerning alcohol is to be construed as equally applicable to other non-solvents which are suitable for this purpose and apparent to those skilled in the art.

It will thus be apparent that our invention is in fact two fold, namely, (1) the bleaching of dyed cellulosic derivative scrap and (2) the leaching of dyed cellulosic derivative scrap prior to the bleaching thereof, the bleaching being optionally followed by further leaching if desired. One is, of course, more or less of a specific subcombination of bleaching included in the broad concept of leaching and bleaching, as the two are quite apparently useful in connection with each other. Those claims appended hereto and directed to bleaching are not, of course, limited to a bleaching preceded by leaching as it may well be employed without previous leaching altho the latter is to be preferred. Also those claims directed more or less broadly to leaching and bleaching are not limited (unless so stated) to a bleaching step including the use of a permanganate as it will be quite apparent that previous leaching will make more easy the majority of bleaching processes such as those disclosed in applications of Charles E. Allen filed of even date, or even the usual hypochlorite or chlorine bleach as disclosed in the Middleton Patent #1,743,155.

Numerous other variations and modifications of the invention will occur to those skilled in the art, and it is intended that all modifications indicated above and which would occur to those skilled in the art shall be included within the spirit of this invention and the scope of the claims appended hereto. For instance, the process is equally applicable to any dyed cellulose derivative waste, such as dyed artificial silk waste which has a base of cellulose nitrate or acetate.

What we claim as our invention and desire to

be secured by Letters Patent of the United States is:

1. The process of reclaiming dyed cellulose derivative film scrap which comprises removing the alcohol soluble components of the scrap by leaching it with a 30-70% aqueous ethyl alcohol solution whereby such components are removed and the scrap is rendered porous, swollen and readily susceptible to further processing, washing the leached scrap to remove residual alcohol, decolorizing the washed material by subjecting it to the oxidizing action of an acid solution of permanganate containing 1-1% of permanganate and thereafter removing the oxidized material from the scrap. 80

2. The process of reclaiming dyed photographic cellulose acetate film scrap which comprises pre-treating the scrap to remove alcohol soluble components and to increase the permeability of the surface layers thereof by leaching with a 30-70% aqueous ethyl alcohol solution, washing the leached scrap with water to remove residual alcohol, decolorizing the washed scrap by subjecting it to the oxidizing action of a 1-1% solution of potassium permanganate, washing the bleached scrap with water and thereafter clearing the scrap from traces of unused permanganate by subjecting it to the reducing action of an acidified solution of sodium bisulphite. 95

3. The process of reclaiming dyed cellulose derivative scrap which comprises removing the alcohol soluble components of the scrap by leaching it with an alcohol which is non-solvent of the film scrap, whereby the alcohol soluble components of the scrap are removed and the scrap is rendered porous, swollen and readily susceptible to further processing, decolorizing the scrap by subjecting it to the oxidizing action of a bleaching solution and thereafter removing from the scrap the products of the oxidation. 105

4. The process of reclaiming dyed cellulose derivative scrap which comprises removing the alcohol soluble components of the scrap by leaching it with an aqueous alcohol which is non-solvent of the film scrap, whereby the alcohol soluble components of the scrap are removed and the scrap is rendered porous, swollen and readily susceptible to further processing, decolorizing the scrap by subjecting it to the oxidizing action of a permanganate solution and thereafter removing from the scrap the products of the oxidation. 120

THOMAS F. MURRAY, JR.  
CYRIL J. STAUD.

Patent No. 1,925,564.

September 5, 1933.

THOMAS F. MURRAY, JR., ET AL.

It is hereby certified that error appears in the printed specification of the above numbered patent requiring correction as follows: Page 2, line 79, claim 1, strike out the word "film"; and that the said Letters Patent should be read with this correction therein that the same may conform to the record of the case in the Patent Office.

Signed and sealed this 28th day of November, A. D. 1933.

F. M. Hopkins

(Seal)

Acting Commissioner of Patents.

**CERTIFICATE OF CORRECTION.**

**Patent No. 1,925,564.**

**September 5, 1933.**

**THOMAS F. MURRAY, JR., ET AL.**

**It is hereby certified that error appears in the printed specification of the above numbered patent requiring correction as follows: Page 2, line 79, claim 1, strike out the word "film"; and that the said Letters Patent should be read with this correction therein that the same may conform to the record of the case in the Patent Office.**

**Signed and sealed this 28th day of November, A. D. 1933.**

**F. M. Hopkins**

**(Seal)**

**Acting Commissioner of Patents.**